

## [54] RENDERING FIBROUS MATERIAL FLAME RETARDANT

[75] Inventors: **Ronald Swidler; William A. Sanderson**, both of Palo Alto; **William A. Mueller**, Pasadena, all of Calif.

[73] Assignee: **Cotton Incorporated**, New York, N.Y.

[22] Filed: **July 2, 1973**

[21] Appl. No.: **375,439**

## Related U.S. Application Data

[63] Continuation-in-part of Ser. No. 259,350, June 2, 1972, abandoned, which is a continuation of Ser. No. 153,094, June 14, 1971, abandoned, which is a continuation of Ser. No. 862,509, Sept. 30, 1969, abandoned.

[52] U.S. Cl. .... **117/136**, 117/139.4, 106/15 FP, 252/8.1

[51] Int. Cl. .... **C09k 3/28**

[58] Field of Search ..... 117/136, 143 A, 139.4, 117/137; 106/15 FP; 252/8.1; 260/502.4 R, 502.4 P, 928, 941, 953, 961

## [56] References Cited

## UNITED STATES PATENTS

|           |         |                    |             |
|-----------|---------|--------------------|-------------|
| 2,530,261 | 11/1950 | Morton et al. .... | 8/116.2     |
| 3,322,716 | 5/1967  | Klein et al. ....  | 260/502.4 R |

Primary Examiner—Charles E. Van Horn

Assistant Examiner—Neal Kalishman

Attorney, Agent, or Firm—Burns, Doane, Swecker & Mathis

## [57] ABSTRACT

Fibrous material such as cotton cloth is rendered flame retardant by treating the material with cyanamide and at least one phosphonic acid represented by the structural formula:



wherein R<sup>1</sup> represents a monovalent radical such as hydrogen or methoxy and R<sup>2</sup> represents a monovalent radical such as hydrogen or methyl. Durability of the flame retardancy to repeated hard water washing may be improved through a subsequent treatment with N-methylo compounds or with additional cyanamide or by methylation with diazomethane. Dimensional stability and durable press properties of cellulosic textiles are also improved by the subsequent treatment with additional cyanamide. A particularly high degree of flame retardancy is imparted to mercerized cotton cloth.

21 Claims, No Drawings

# RENDERING FIBROUS MATERIAL FLAME RETARDANT

## CROSS REFERENCE TO RELATED APPLICATIONS

This is a continuation in part of copending application Ser. No. 259,350, filed June 2, 1972, now abandoned which in turn is a continuation of application Ser. No. 153,094, filed June 14, 1971, now abandoned, which in turn is a continuation of Ser. No. 862,509, filed Sept. 30, 1969, now abandoned.

## BACKGROUND OF THE INVENTION

## 1. Field of the Invention

This invention relates to flame retardant fiber-containing material and to processes for producing the same.

## 2. State of the Art

Natural fiber-containing textile materials such as cotton cloth have been employed since ancient times. However, the combustibility of these textile materials has inhibited their wider use in certain instances. A great number of flame retardants have been proposed for use with cellulosic textile materials, but these flame retardants suffer from one or more disadvantages.

A major disadvantage of many prior flame retardants is their lack of wash fastness or durability, by which is meant that while they initially render the cellulosic textile material flame retardant, such flame retardancy disappears after one or more household launderings, especially in hard water. This phenomenon is described by O'Brien in "Cyanamide-Based Durable Flame-Retardant Finish for Cotton," *Textile Research Journal*, Mar. 1968, pp. 256-266. This article describes the treatment of cellulosic textile materials with flame retardants of cyanamide and phosphoric acid. However, the flame retardants disclosed therein by O'Brien are not resistant to hard water washing. Similarly, East German Pat. Nos. 15,357 and 18,253, and Schiffner et al. in *Faserforsch u. Texiltech.*, 14, (9), 375-86 (1963) describe specific attempts to impart flame resistance to textile material with certain flame retardants, including combinations of urea or dicyandiamide with chloromethyl phosphonic acid, or urea with hydroxymethyl phosphonic acid, which combinations may also not be resistant or durable to repeated cycles of hard water washings, or which may unduly degrade the physical strengths of fabrics.

Other disadvantages include the relatively large quantities (high add-on) which may be necessary in order to impart flame retardance, and the undesirable alteration of other properties of the cellulosic textile material such as color, hand, and susceptibility to dyeing.

Also, many flame retardants are incompatible with commonly employed crease-proofing agents; in the past this limitation has discouraged use of flame retardants in conjunction with a crease-proofing operation so as to yield a textile material which is both flame retardant and wrinkle resistant.

## SUMMARY OF THE INVENTION

Accordingly, a primary object of the present invention is to render fiber-containing material flame retardant while preventing or substantially alleviating one or more of the above-discussed disadvantages of prior processes.

Another object is to provide an improved process for imparting flame retardancy to cellulosic textile materials which flame retardancy is durable and resistant to multiple household launderings in general and especially in hard water.

Another object is to provide an improved cellulosic flame-retarding process requiring only a relatively small add-on or amount of flame retardants.

A still further object is to provide an improved process for rendering cellulosic textile material flame retardant which does not adversely affect the other properties of the material.

Another object of the present invention is to provide a cellulosic flame-retarding process having improved efficiencies of reaction between the flame retardants and the cellulosic material.

Yet another object is to provide an improved process for rendering cellulosic textile material both flame retardant and wrinkle resistant, with improved dimensional stability.

Yet another object is to provide flame resistant fibrous products produced by these processes.

Additional objects and advantages of the present invention will be apparent to those skilled in the art by reference to the following summary of the characteristic features of the present invention and the subsequent description of the preferred embodiments:

In accordance with a primary aspect of the present invention, a process is provided for rendering cellulosic and wool fiber-containing material flame retardant comprising contacting the material with cyanamide and at least one phosphonic acid represented by the structural formula:



40 to deposit or fix on the material a flame-retarding amount of the phosphonic acid with cyanamide. In the above formula,  $R^1$  represents a monovalent radical such as hydrogen and  $R^2$  represents a monovalent radical such as methyl or hydrogen.

45 A central feature of the present invention is the discovery that cyanamide and the above described phosphonic acids can impart durable, hard water wash-resistant, flame retardancy to cellulosic fiber-containing material, particularly mercerized cotton cloth. In addition, the fire retardancy-imparting systems of the present invention have improved efficiencies in terms of efficiency of reaction between the flame retardants and the cellulose, and in terms of fire retardancy per unit add-on of phosphorus.

In accordance with another aspect of the present invention, the fibrous material rendered flame-retardant as indicated above is subsequently treated to improve the durability of flame retardancy to repeated hard water washing by contacting the material with additional cyanamide. Also, this subsequent treatment with additional cyanamide has been found to improve dimensional stability and durable press properties of cellulosic textile material.

55 In accordance with yet another aspect of the present invention, durability of the flame retardancy of the fibrous material to repeated hard water washing is improved by methylation of the acid form of the phos-

phonic acid residue on the fibrous material. In a preferred embodiment described below, such methylation is accomplished by contacting the fibrous material with diazomethane.

In accordance with another aspect of the present invention, the fibrous material rendered flame retardant by the phosphonic acid and cyanamide as indicated above is subsequently treated to improve the durability of flame retardancy to repeated hard water washing by contacting the material with at least one water-soluble, compound possessing reactive N-methylol groups, and thereafter curing the material to fix or insolubilize the compound on the material.

Other aspects and advantages of the present invention will be apparent to one skilled in the art from the following:

#### DESCRIPTION OF THE PREFERRED EMBODIMENTS

As indicated above, cyanamide (HNCNH or H<sub>2</sub>NCO), also known as carbodiimide, is used along with certain phosphonic acids to impart the wash-resistant flame retardancy to the fibrous or fiber-containing material.

The phosphonic acids which may be suitable can be represented by the general structural formula:



where R<sup>1</sup> represents a monovalent radical such as hydrogen or lower alkoxy, and R<sup>2</sup> represents a monovalent radical such as hydrogen or lower alkyl. The alkyl radicals or portions of the radicals may contain, for example, from 1 to 4 carbon atoms.

Non-limiting examples of phosphonic acids having the above-described structural formula and which may be used according to the process of the present invention including methyl phosphonic acid, methyl phosphonic acid monomethyl ester, methoxymethyl phosphonic acid, and methoxymethyl phosphonic acid monomethyl ester. Mixtures of two or more of the phosphonic acids may be used if desired.

The more preferred phosphonic acids are methyl phosphonic acid and methyl phosphonic acid monomethyl ester, and the most preferred phosphonic acid is methyl phosphonic acid insofar as it has been found to give or impart the most durable flame retardancy to the cellulosic materials.

The manner in which the phosphonic acids and cyanamide are prepared or derived is per se well known and does not form a part of the present invention.

The cellulosic and wool fiber-containing materials which may be treated according to the present invention are generally any of those which have been previously employed in conjunction with known flame retardants. The fiber-containing or textile material can have a wide variety of physical forms and can be fibers, filaments, yarns, threads, and particularly woven and non-woven cloth. The cellulosic fiber material can be cotton, flax, linen, hemp, or regenerated cellulose such as rayon (e.g., viscose rayon). Mercerized cotton may give particularly advantageous results. (Mercerized cotton is well known per se; mercerization typically comprises passing cotton through a 25 to 30 percent

solution of sodium hydroxide under tension, and then washing the cotton with water while under tension. Mercerization using liquid ammonia is also known). These fiber-containing or textile materials can be mixtures of two or more different fibers, e.g., a mixture of cellulosic fibers with other fibrous materials such as nylon (e.g., nylon 6, 6), polyester (e.g., polyethylene terephthalate), acrylics (e.g., polyacrylonitrile), polyolefins (e.g., polypropylene), polyvinyl chloride, polyvinylidene chloride, and polyvinyl alcohol fibers.

The preferred cellulosic textile materials are those containing 50 weight percent or more of cotton and especially pure, i.e., essentially 100 weight percent, cotton cloth.

According to a broad aspect of the present invention, fire or flame retardancy can be imparted to fibrous material by simply contacting or impregnating the material with the phosphonic acid and cyanamide under widely varying conditions of temperature and pH. However, durable, i.e., wash resistant, flame retardancy is imparted only by fixing, i.e., reacting, the phosphonic acid with the cyanamide on the material. This fixing or "curing" is generally accomplished by heating the treated material at superambient temperatures and at low pH. Broadly, any temperature can be employed above which the phosphonic acid and cyanamide are fixed or reacted on the material and below which undesirable thermal degradation of the material begins, and generally from 20° to 400°C and preferably from 100° to 300°C. Optimum results are obtained at 120° to 180°C.

Durable flame retardance is imparted if, concurrently with the above described heating, the pH of the reacting mixture on the material is low, i.e., typically less than 2.5 and preferably less than 1.5, e.g., about 1.0. While these pH's are believed to be critical to durability it is generally valid to assume that the pH of the reacting mixture on the material is the same as the pH of the mixture of phosphonic acid, cyanamide, and solvent when present, except as indicated below for the in situ generation of the reactants.

The fibrous material may be contacted with a simple mixture of the phosphonic acid and cyanamide; and a solvent is preferably present. The solvent can be employed in any amount up to infinite dilution as long as the final treated material has an add-on sufficient to impart flame retardancy, which add-on may be, for example, from 2 to 15 weight percent. Add-on is defined and used herein as the increase ("dry" basis) in weight of the fibrous material due to the addition of the flame retardant as a percentage of the weight of the untreated fibrous material. Examples of suitable solvents include lower alkanols such as methanol and ethanol, lower alkylene or alkyl ethers such as dioxane and ethyl ether, or, most preferably, water. Such solutions are termed pad baths.

The fibrous material can be contacted with the phosphonic acid and cyanamide sequentially but is preferably contacted with both simultaneously.

This mixture of phosphonic acid and cyanamide can be employed at autogenous pH which is generally about 0.8 or at a slightly higher pH, e.g., about 1.0 to 1.5, except as indicated below for the in situ generation of the reactants where the pH of the pad bath may vary up to about 6.0. Naturally, in the latter case the pH of the pad bath may be quite different than the pH on the material at fixation.

A method by which the above described phosphonic acids can be formed in situ is by the thermal degradation of the corresponding ammonium salt such as mono- or di-ammonium methyl phosphonic acid, or ammonium methyl phosphonic acid monomethyl ester. For example, ammonium hydroxide can be added to a pad bath containing the phosphonic acid (which would, of course, raise the pH, typically to about 3.0). Thus, in the fixing step there is initially present, on the fibrous material, cyanamide and an ammonium salt of the phosphonic acid. Upon heating to fixation, the ammonium salt would decompose to ammonia and the corresponding phosphonic acid (resulting in a lowered pH). Usage of such ammonium salts and the inherent raising of the pH of the pad bath can be advantageous where lower pH (higher acidity) pad baths are not desired due to corrosion and personnel handling considerations.

In a preferred process for rendering fibrous materials such as cellulosic textile materials flame retardant according to the present invention, the material is first contacted with an aqueous solution comprising a mixture of phosphonic acid and cyanamide at the desired pH in a molar ratio of 1:10 to 10:1, preferably 1:2 to 3:1, and most preferably 1:2 to 2:1. The excess solution is then removed from the material by any suitable means such as by passing the material between the nip of two rollers. The material is then dried to remove excess water. The drying can be accomplished at any temperature but is generally accomplished at superambient temperatures and preferably from 20° to 150°C. The material is then heated in order to fix the phosphonic acid and cyanamide on the material and is conducted at the above described fixation temperatures. The heating is conducted for at least several seconds and up to several hours, more typically from one to 15 minutes. In certain instances, the fixing may be generally complete in within 2 to 10 minutes. The drying and heating steps can be conducted simultaneously but are preferably conducted sequentially. The fixing of the phosphonic acid with the cyanamide on cellulosic material is presently thought to occur in the form of a reaction product which then reacts with the hydroxyl groups of the cellulosic material.

The treated fibrous material preferably has sufficient add-on such that it exhibits the desired degree of flame retardancy. Such materials generally have add-ons of 1 to 30, and preferably 10 to 20 percent.

It is only critical to the present invention that the above described phosphonic acids and cyanamide be present on the fibrous material. Therefore, according to another embodiment of the present invention many of these compounds can be formed in situ. A preferred method by which the above described phosphonic acids can be formed in situ is by the above-described thermal degradation of the corresponding ammonium salt such as ammonium methyl phosphonic acid monomethyl ester, or mono- or di-ammonium methyl phosphonic acid. Another method which involves thermally decomposable esters which upon heating yield the above-described phosphonic acids can be employed. Examples of such esters include among others methyl phosphonic acid mono-t-butyl ester and methyl phosphonic acid monomethyl ester mono-t-butyl ester. These compounds thermally decompose to give respectively methyl phosphonic acid and methyl phosphonic acid monomethyl ester. A third method may be by the use of metal salts of the phosphonic acids together with

means for creating the low pH's necessary to effect fixation. For example, the pH of the pad bath may be increased with sodium hydroxide, followed by the addition of ammonium chloride. Thus, in the fixing step there would be present on the cellulosic material; cyanamide, a sodium salt of the above described phosphonic acids, and ammonium chloride. Upon heating, the ammonium chloride would decompose to ammonia and hydrochloric acid converting the sodium salt to the free acid to accomplish fixation. Naturally, in these cases the pH of the pad may be quite different than the pH on the material.

The solution of phosphonic acid and cyanamide into which the cellulosic material is dipped may also contain, if desired, conventional softeners, lubricants, stiffeners, brighteners, water-repellants, soil release agents, and dyes.

The fibrous material rendered flame retardant as indicated above may be subsequently processed to improve durability of the flame retardancy by treating the material with additional cyanamide, or diazomethane (methylation), or water-soluble compounds possessing reactive N-methylol groups. When such further processing or "retreatments" are employed, the acid form of the phosphonic acid residue typically needs to be regenerated such as by contacting or "souring" with a dilute hydrochloric acid solution. Such regeneration is typically necessary due to what is thought to be inherent chemical breakdown of cyanamide to produce eventually ammonia in the curing or fixation state, which results in an ammonium salt form of the phosphonic acid residue on the fabric. And after hard water washing, the phosphonic acid residues may inherently be present on the fabric as their calcium salts, as further explained hereinbelow.

After laundering in hard water, the phosphonic acid residues are thought to be at least in part present on the fabric as their calcium salts, e.g.,



And generally, for a given phosphonic acid the order of flame retardant efficiency (char length) is acid > monomethyl ester > calcium salt. It is thought that this subsequent retreatment with cyanamide causes further reaction of the phosphonic acid residue with the fiber-containing material, which further reaction lowers ionicity and therefore lowers susceptibility to calcium pickup (increases resistance to ion exchange) during hard water washings. As a consequence, flame retardance, and especially the durability of flame retardance, is improved.

In the case of cellulosic textile materials, the further reaction of the phosphonic acid by the cyanamide is thought to be in the nature of a crosslinking reaction insofar as, surprisingly, dimensional stability or shrinkage control, durable press properties (wrinkle resistance), and overall shape retention and wash/wear properties are also demonstrably improved.

When cyanamide is used in this subsequent treatment, the acid form of the phosphonic acid residue should be regenerated such as by contacting or "souring" with a dilute hydrochloric acid solution, and the soured fibrous material is then contacted or impreg-

nated with cyanamide as generally indicated above for the initial flame retardancy treatment. For example, the material may be contacted with a solution of cyanamide. Examples of suitable solvents include methanol, ethanol, dioxane and, most preferably, water. The cyanamide is present in the solution or pad bath in an amount sufficient to improve flame retardancy (or reduce ionicity) as discussed above. For example, the concentration of cyanamide in solution may range from about 1 to 50 weight percent, and more typically, from 10 to 20 weight percent. Higher or lower concentrations may be used if desired.

As in the initial treatment, any excess solution may then be removed from the fibrous material by any suitable means such as by passing the material between the nip of two rollers. The material may then be dried to remove excess water. The drying can be accomplished at any temperature but is generally accomplished at ambient or superambient temperatures, and preferably from 20° to 150°C. The material with the cyanamide is then heated in order to further react the phosphonic acid residue on the fibrous material. Broadly, any temperature can be employed above which the phosphonic acid residue is further reacted with the material by the cyanamide and below which undesirable thermal degradation of the material begins, and generally from about 50° to 400°C, preferably from 100° to 300°C, and most preferably from 120° to 180°C. The heating is conducted for at least several seconds up to several hours, more typically from about 10 seconds to 2 hours and preferably from about one to 15 minutes. The drying and heating steps can be conducted simultaneously but are preferably conducted sequentially.

As indicated above, the treated material preferably has sufficient add-on such that it exhibits the desired degree of flame retardancy. Such materials generally have add-ons of about 1 to 30, and preferably about 10 to 20 percent.

When diazomethane is used in the subsequent treatment, the acid form of the phosphonic acid residue should be regenerated such as by contacting or "souring" with a dilute hydrochloric acid solution, and the soured fibrous material is contacted with diazomethane as generally indicated above for subsequent treatment with cyanamide. For example, the fibrous material may be contacted, e.g., immersed, in an ether solution of diazomethane for about 1 to 2 hours at 0° to 30°C. Such treatment with diazomethane is thought to bring about methylation of the phosphonic acid residue, thus reducing ionicity and calcium pickup (increasing resistance to ion exchange), and improving flame retardancy, especially durable flame retardancy. Other methylating agents such as orthoesters, e.g., trimethyl orthoformate, may also be used to bring about methylation of the phosphonic acid residue. These methylating agents are well known per se and their production or derivation is not part of the present invention.

When one or more N-methylol compounds are used in the subsequent treatment, the acid form of the phosphonic acid residue should be regenerated such as by contacting or "souring" with a dilute hydrochloric acid solution, and the soured fibrous material is contacted with the N-methylol compound and is thereafter cured to fix or insolubilize the compound on the material.

The water-soluble compounds possessing reactive N-methylol groups, sometimes referred to herein as N-methylol compounds, include the substantially water

soluble precondensates which are obtained by condensation of formaldehyde with a compound such as melamine or a lower alkylsubstituted melamine, or a urea. The resulting methylol-containing compound or precondensate may be further etherified by reaction with a lower alkanol such as methanol or butanol. As is well known in the fabric treating art, these precondensates are capable of being applied to fibrous materials from an aqueous solution. Good results may be obtained, for example, using precondensates obtained by condensing 1 mole of melamine or an alkyl substituted melamine with 1 to 6 moles of formaldehyde, i.e., using mono-, di-, tri-, tetra-, penta-, or hexa-methylol melamine. Such products function well to increase flame retardancy durability and can be readily fixed or cured on fibrous material by heating as described herein. Commercially available products of this kind include Aerotex 23, an alkylated melamine-formaldehyde precondensate, Aerotex M-3, a dimethoxymethyl hydroxymethyl melamine; Aerotex P-225, a hexakis (methoxymethyl) melamine; Aerotex 19, which is a less completely fractionated modification of Aerotex P-225, and Aerotex 92 which is a melamine having an average of about 1.5 methylol groups. These Aerotex products are supplied by American Cyanamide Company. Equivalent products are commercially available from other manufacturers such as Monsanto Company which produces Resloom HP, which is a melamine having an average of about 2 to 3 methylol groups. To be applied by padding, one or more of the aforementioned N-methylol compounds may be dissolved in water to form a solution containing from about 1 to 50%, preferably about 5 to 20%, N-methylol compound. To facilitate insolubilization or formation of polymer on the fabric in a desired amount, it may be desirable in certain cases to add to the padding solution, a catalyst such as formic acid, citric acid, hydrochloric acid, or, particularly, an acid-acting salt such as zinc nitrate, zinc chloride, magnesium chloride, ammonium chloride, aluminum chloride, sodium hydrogen phosphate, or sodium dihydrogen phosphate. Such a catalyst may be added to the pad bath in a concentration of between about 0.1 and 10% by weight of the N-methylol compound. Formation of the water-insoluble form of the N-methylol compound on the fibrous material is typically aided by heat in addition to acidity. After application of the N-methylol compound to the fibrous material, the latter is dried and finally cured under conditions essentially the same as or similar to those described earlier herein in connection with the subsequent treatment with cyanamide.

Application of the N-methylol compound-containing solution to the fibrous material may be done by conventional padding using customary equipment, or by other processes well known in the art. Typically, the solutions are applied to the fibrous materials in a wet pickup of from about 40 to 120%, so as to give upon fixation an add-on of between about 1 and 15%, based on dry fabric weight. The padding may be conducted at ambient temperature, e.g., between about 10° and 30°C. As in the initial treatment, any excess solution may then be removed from the fibrous material by any suitable means such as by passing the material between the nip of two rollers. The material may then be dried to remove excess water. The drying can be accomplished at any temperature but is generally accomplished at ambient or superambient temperatures, and

typically from 20° to 100°C. The material with the N-methylol compound is then heated in order to fix or insolubilize the N-methylol compound on the fibrous material. Broadly, any temperature can be employed above which the N-methylol compound is reacted on the material and below which undesirable thermal degradation of the material begins, and preferably from 100° to 300°C, and most preferably from 120° to 180°C. The heating is conducted for at least several seconds up to several hours, more typically from about 10 seconds to 2 hours and preferably from about one to 15 minutes. The drying and heating steps can be conducted simultaneously but are preferably conducted sequentially.

Such treatment with N-methylol compounds has been found to reduce ionicity and calcium pickup (increasing resistance to ion exchange), thus improving durable flame retardancy. Increased durability of flame retardancy through such subsequent treatment with N-methylol compounds was unexpected insofar as the utilization of such compound in the initial pad baths containing the phosphonic acid and cyanamide reduced flame retardancy. Moreover, other conventional creaseproofing agents such as dimethylol dihydroxy ethylene urea have been found not to increase significantly the durability of flame retardancy.

If desired, more than one subsequent treatment with additional cyanamide or diazomethane or N-Methylol compound may be used. Combinations of subsequent treatments with diazomethane and N-methylol compound and retreatments with cyanamide may also be used if desired.

The present invention is further illustrated by the following examples; all parts and percentages in the examples as well as in other parts of the specification and claims are by weight unless otherwise indicated. These non-limiting examples are illustrative of certain embodiments designed to teach those skilled in the art how to practice the invention and to represent the best mode contemplated for carrying out the invention.

#### EXAMPLE I

This example illustrates the process of the present invention employing cyanamide and methyl phosphonic acid (MPA) or methoxy methyl phosphonic acid

(MMPA) in aqueous solutions of varying acid to cyanamide molar ratios as is shown in TABLE I. Comparison runs 8 to 14 were also made using cyanamide and chloromethyl phosphonic acid (CMPA) or hydroxymethyl phosphonic acid (HMPA) in aqueous solutions of varying acid to cyanamide weight ratios as shown in TABLE I.

For each run, a weighed piece of cotton twill measuring 12 inches × 12 inches was dipped into the aqueous solution or "pad bath" of cyanamide and phosphonic acid and then passed between the nip of two rollers to remove the excess solution. The cloth was then dried in an oven for 10 minutes at 80°C and then cured (fixed) in a second oven for 15 minutes at 160°C. The fabric was then washed once as described below, dried, conditioned at 65% relative humidity at 21°C and reweighted. The difference between the initial weight of the sample prior to the contact with the solution and final weight of the cloth after one wash divided by the initial weight of the cloth times 100 is recorded in TABLE I as "add-on." This procedure was repeated for each of the remaining solutions.

Each of the samples was then washed the indicated number of times in an automatic home laundering machine having one wash and two rinses with intermediate spin dry operations. A hard water solution of household laundry detergent, commercially available as "ALL Laundry Detergent," was employed as the wash water (pH 8.5). Hard water was employed in the rinses. In this example, the term "hard water" refers to Irvine, Calif., water containing a degree of hardness equivalent to 350-380 ppm of calcium carbonate. Total dissolved solids amount to 750-850 ppm. The flame retardancy was then measured according to American Association of Textile Chemists and Colorists (AATCC) procedure 34-1966 and the char length in inches is shown in TABLE I. (The greater the char length, the less the flame retardancy.) A qualitative pass (+)/fail (-) vertical strip-match test was also given to each of the treated samples.

As may be seen from TABLE I, at the optimum MPA: cyanamide ratio of 1:2 (run 2) the retardance is durable for at least 250 washes. At an MMPA:cyanamide ratio of 1:2 (run 6) the retardance is durable for at least 50 washes.

TABLE I

| Run No. | Acid Used | Cyanamide in Bath (%) <sup>1</sup> | Acid:Cyanamide Ratio | Add-On (%) | P (%) | N (%) | Cl (%) | Fill Strength Retention (%)<br>(One Wash) |                     |
|---------|-----------|------------------------------------|----------------------|------------|-------|-------|--------|-------------------------------------------|---------------------|
|         |           |                                    |                      |            |       |       |        | Tear                                      | Tensile             |
| 1       | MPA       | 8                                  | 1:1                  | 13.6       | 2.46  | 0.47  | —      | 116                                       | 58                  |
| 2       | MPA       | 16                                 | 1:2                  | 17.7       | 3.28  | 0.61  | —      | 94                                        | 55                  |
| 3       | MPA       | 24                                 | 1:3                  | 17.2       | 2.94  | 0.87  | —      | 97                                        | 55                  |
| 4       | MPA       | 48                                 | 1:6                  | 14.6       | 2.25  | 1.42  | —      | 127                                       | 64                  |
| 5       | MMPA      | 8                                  | 1:1                  | 10.2       | 1.62  | 0.52  | —      | —                                         | —                   |
| 6       | MMPA      | 16                                 | 1:2                  | 16.1       | 2.54  | 0.71  | —      | —                                         | —                   |
| 7       | MMPA      | 24                                 | 1:3                  | 17.1       | 2.42  | 0.87  | —      | —                                         | —                   |
| 8       | CMPA      | 8                                  | 1:1                  | 12.2       | 1.89  | 0.70  | 1.95   | 71                                        | 43                  |
| 9       | CMPA      | 16                                 | 1:2                  | 16.8       | 2.49  | 1.01  | 2.24   | 67                                        | 63                  |
| 10      | CMPA      | 24                                 | 1:3                  | 17.8       | 2.53  | 1.49  | 1.60   | 87                                        | 56                  |
| 11      | CMPA      | 32                                 | 1:4                  | 20.4       | 2.46  | 2.72  | 1.22   | 72                                        | 55                  |
| 12      | CMPA      | 48                                 | 1:6                  | 24.0       | 2.25  | 3.30  | 1.08   | 77                                        | 60(50) <sup>2</sup> |
| 13      | HMPA      | 8                                  | 1:1                  | 11.4       | 2.17  | 0.80  | —      | —                                         | —                   |
| 14      | HMPA      | 16                                 | 1:2                  | 18.7       | 3.16  | 0.90  | —      | —                                         | —                   |

Flame Retardance = Char Length (in.) and Match Test<sup>3</sup> at Number of Washes Shown ("ALL" Detergent)

| Run No. | 1      | 5      | 10     | 20     | 40     | 50     | 80     | 150   | 250   |
|---------|--------|--------|--------|--------|--------|--------|--------|-------|-------|
| 1       | 2½ (-) | 3¼ (-) | 3¼ (-) | BEL    | —      | —      | —      | —     | —     |
| 2       | 1¾ (+) | 2 (+)  | 2 (-)  | 2 (-)  | 2 (-)  | 2 (-)  | 2 (-)  | 2 (-) | 2 (-) |
| 3       | 1½ (+) | 2¼ (±) | 2½ (±) | 3¼ (-) | 2¼ (-) | 2¼ (-) | 2½ (-) | BEL   | —     |

TABLE I—Continued

| Run No. | Flame Retardance = Char Length (in.) and Match Test <sup>a</sup> at Number of Washes Shown ("ALL" Detergent) |           |           |                  |           |           |           |     |     |
|---------|--------------------------------------------------------------------------------------------------------------|-----------|-----------|------------------|-----------|-----------|-----------|-----|-----|
|         | 1                                                                                                            | 5         | 10        | 20               | 40        | 50        | 80        | 150 | 250 |
| 4       | 2 (+)                                                                                                        | —         | 2 1/4 (-) | 2 (-)            | 2 1/4 (-) | 2 1/2 (-) | —         | —   | —   |
| 5       | BEL                                                                                                          | —         | —         | —                | —         | —         | —         | —   | —   |
| 6       | 3 1/4 (-)                                                                                                    | —         | —         | 3 1/4 (-)        | 3 1/4 (-) | 3 1/4 (-) | —         | —   | —   |
| 7       | 2 1/2 (+)                                                                                                    | —         | —         | 3 1/4 (-)        | 3 1/4 (-) | 3 1/4 (-) | —         | —   | —   |
| 8       | BEL                                                                                                          | —         | —         | —                | —         | —         | —         | —   | —   |
| 9       | 1 3/4 (±)                                                                                                    | 2 1/4 (-) | 3 (-)     | BEL <sup>b</sup> | —         | —         | —         | —   | —   |
| 10      | 1 1/4 (+)                                                                                                    | 1 1/2 (+) | 2 (-)     | 2 (-)            | 2 (-)     | 2 1/4 (-) | 2 1/2 (-) | BEL | —   |
| 11      | 1 1/2 (+)                                                                                                    | —         | —         | 2 (±)            | 2 1/4 (±) | 3 (±)     | —         | —   | —   |
| 12      | 1 1/4 (+)                                                                                                    | —         | 1 1/4 (+) | 2 1/2 (+)        | 1 1/4 (±) | 2 (±)     | —         | —   | —   |
| 13      | BEL                                                                                                          | —         | —         | —                | —         | —         | —         | —   | —   |
| 14      | 2 1/2 (-)                                                                                                    | —         | —         | BEL              | —         | —         | —         | —   | —   |

<sup>a</sup>The bath also contained, in addition to the cyanamide and phosphonic acid, 0.1 percent Triton X-100 non-ionic wetting agent and 5 percent Velvamine 380 polyethylene softeners.

<sup>b</sup>Value in parentheses measured in area of char.

<sup>c</sup>(+) = passed match test; (-) = failed match test; (±) = burned greater than 3 inches but not entire length.

<sup>d</sup>In a substantially duplicate run where higher percentages of P, N and Cl were recorded, as well as a lower degree of ionicity, the flame retardance at fifty washes was 2 3/4 (-).

## EXAMPLE II

This example illustrates the process of the present invention employing cyanamide and methyl phosphonic acid in solutions of varying pH. In this example, the term "hard water" refers to Pasadena, Calif., water containing a degree of hardness equivalent to 128 ppm of calcium carbonate. Total dissolved solids amount to 236 ppm.

The following quantities of the following ingredients were combined as indicated:

| Ingredient                                   | Grams | Quantity | Moles |
|----------------------------------------------|-------|----------|-------|
| methyl phosphonic acid                       | 48    |          | 0.5   |
| cyanamide (84g of 50 wt. % aqueous solution) | 42    |          | 1.0   |
|                                              |       |          |       |

The phosphonic acid and cyanamide were mixed with an amount of water added to the mixture to give a total volume of 300 ml of solution containing 30 percent solids and having a pH of 0.8. This solution was divided into six 50 ml samples and the pH of each adjusted to the value shown in Column 2 of TABLE II of

20 second oven for 15 minutes at 160°C. The fabric was then washed once as described below, dried, conditioned at 65 percent relative humidity at 21°C and reweighed. The difference between the initial weight of the fabric sample prior to the contact with the solution and final weight of the cloth after one wash divided by the initial weight of the cloth times 100 is recorded at Column 3 of TABLE II, as "add-on." This procedure was repeated for each of the remaining solutions.

Each of the fabric samples was then washed the indicated number of times in an automatic home laundering machine having one wash and two rinses with intermediate spin dry operations. A hard water solution of alkyl benzene sulfonate, commercially available as "Sears Super-concentrated Laundry Detergent," was employed as the wash water (pH 10.3). Hard water was employed in the rinses. The flame retardancy was then measured according to American Association of Textile Chemists and Colorists (AATCC) procedure 34-1966 and the char length in inches is shown in Columns 4 through 8 of TABLE II. (The greater the char length, the less the flame retardancy.)

As may be seen from TABLE II, at a pH of 1.0 (run 15) the flame retardance was durable for at least 30 washes.

45

TABLE II

| Run No. | pH  | Add On (Approx.) (wt. %) | AATCC 34-1966 (length of char) |                   |                  |                     |                     |
|---------|-----|--------------------------|--------------------------------|-------------------|------------------|---------------------|---------------------|
|         |     |                          | one wash (in.)                 | five washes (in.) | ten washes (in.) | twenty washes (in.) | thirty washes (in.) |
| 15      | 1.0 | 9.1                      | 2 1/2                          | 4                 | 4                | 3 3/4               | 4                   |
| 16      | 1.5 | 8.3                      | 2 1/4                          | 4 1/4             | 4 1/4            | 4 1/4               | BEL                 |
| 17      | 2.0 | 8.2                      | 3 1/4                          | BEL               | —                | —                   | —                   |
| 18      | 2.5 | 5.0                      | 3 1/4                          | BEL               | —                | —                   | —                   |
| 19      | 3.0 | 4.3                      | BEL                            | —                 | —                | —                   | —                   |
| 20      | 3.5 | 2.3                      | BEL                            | —                 | —                | —                   | —                   |

### Legend

BEL = burned entire length

the following table with 50 wt. % NaOH.

For each run, a weighed piece of cotton twill measuring 12 inches × 12 inches was dipped into a solution sample and then passed between the nip of two rollers to remove the excess solution. The cloth was then dried in an oven for 10 minutes at 80°C and then cured in a

## EXAMPLE III

65 This example illustrates certain preferred embodiments of the present invention employing cyanamide with methyl phosphonic acid monomethyl ester and gives a comparison to the use of cyanamide with chlo-

romethyl phosphonic acid monomethyl ester.

The procedure of Example II is repeated employing the same quantities of the same ingredients and the same times, procedures and conditions with the exception that the methyl phosphonic acid is replaced by methyl phosphonic acid monomethyl ester in runs 21-24 and with chloromethyl phosphonic acid monomethyl ester in comparison runs 25-27, with varying percentages of acid and cyanamide in the bath. Data and results are recorded in TABLE III. In TABLE III the values in Column 12 are calculated by the formula:

| Fill       | 100 | Tensile strength after treatment  |
|------------|-----|-----------------------------------|
| Strength = |     | Tensile strength before treatment |

The values of tensile strength are determined according to ASTM D1682-59T and are measured in the "fill" direction of the material. The fill direction is also known as the direction parallel to the woof threads.

As may be seen from TABLE III, at a pH of from 0.5 to 1.0 (runs 21-22), flame retardance was durable for at least 50 washes for methyl phosphonic acid monomethyl ester.

parison to the effect of mercerization of the cotton (flannel) fabric.

The procedure of Example 1, run 2, is repeated employing the same quantities of the same ingredients and the same times, procedures and conditions with the exception that unmercerized flannel cloth (Barium No. -100) was used for run 28 and mercerized flannel cloth (Barium No. -154) was used in run 29, and except that soft water (Menlo Park, California) containing a degree of hardness equivalent to 20 ppm of calcium carbonate was used instead of the Irvine water. The results are recorded in TABLE IV.

As may be seen from TABLE IV, the flame retardancy for the mercerized flannel (run 29 was durable for at least 50 washes.

Mercerization of cotton is believed to increase the number of anhydroglucose units available for reaction, i.e., "removes" them from relatively inpenetrable crystalline regions of the cellulose. Thus, when a given amount of flame retardancy-imparting reactants is applied to the cellulose, the concentration of reactive sites on a mercerized fabric is greater relative to a simi-

TABLE III

FLAME RETARDANCE OF MPAM:CYANAMIDE  
AND CMPAM:CYANAMIDE SYSTEMS

| Run No. | Acid Used | Acid in Bath (%) | Cyanamide in Bath (%) | pH  | Add On (wt %) | Flame Retardance after Indicated Number of Washes AATCC 34-1966 (length of char) |                   |                     |                     |                    |                    | Fill Strength Retention (%) |
|---------|-----------|------------------|-----------------------|-----|---------------|----------------------------------------------------------------------------------|-------------------|---------------------|---------------------|--------------------|--------------------|-----------------------------|
|         |           |                  |                       |     |               | one wash (in.)                                                                   | five washes (in.) | twenty washes (in.) | thirty washes (in.) | forty washes (in.) | fifty washes (in.) |                             |
| 21      | MPAM      | 33               | 25                    | 0.5 | 12.2          | 3                                                                                | 3 1/4             | —                   | —                   | —                  | 4 1/4              | 72                          |
| 22      | MPAM      | 33               | 25                    | 1.0 | 11.2          | 3                                                                                | 3 1/4             | 4                   | —                   | —                  | 4                  | —                           |
| 23      | MPAM      | 31               | 24                    | 2.0 | 11.1          | 3 1/2                                                                            | —                 | 4                   | 4 1/2               | BEL                | —                  | 94                          |
| 24      | MPAM      | 31               | 24                    | 3.0 | 8.1           | 4                                                                                | BEL               | —                   | —                   | —                  | —                  | —                           |
| 25      | CMPAM     | 41               | 24                    | 1.0 | 16.4          | 2 1/2                                                                            | 3 1/4             | 4 1/2               | BEL                 | —                  | —                  | —                           |
| 26      | CMPAM     | 38.5             | 22.5                  | 2.0 | 11.0          | 3 1/2                                                                            | BEL               | —                   | —                   | —                  | —                  | —                           |
| 27      | CMPAM     | 36               | 21                    | 3.0 | 9.0           | 4 1/4                                                                            | BEL               | —                   | —                   | —                  | —                  | —                           |

## Legend

MPAM = methyl phosphonic acid monomethyl ester

CMPAM = chloromethyl phosphonic acid monomethyl ester

BEL = burned entire length

## EXAMPLE IV

This example illustrates certain preferred embodiments of the present invention employing cyanamide with methyl phosphonic acid (MPA) and gives a com-

lar but unmercerized fabric, and hence, the efficiency of immobilization is increased (i.e., wash-off is decreased). This phenomena is significant insofar as efficiencies of reactants, durability of flame retardancy, 50 and overall process economies are improved.

TABLE IV

EFFECT OF MERCERIZATION ON FLAME RETARDANCE  
(METHYL PHOSPHONIC ACID:CYANAMIDE)

Flame Retardance After Indicated Number

| Run No. | Acid Used | Add On (wt %) | Mercerized | N(%)<br>(One Wash) | P(%)<br>(One Wash) | of Washes AATCC 34-1966 (length of char) |                    |
|---------|-----------|---------------|------------|--------------------|--------------------|------------------------------------------|--------------------|
|         |           |               |            |                    |                    | One Wash (in.)                           | Fifty Washes (in.) |
| 28      | MPA       | 15.7          | No         | 0.48               | 3.26               | 2 1/4 (-)                                | BEL                |
| 29      | MPA       | 25.4          | Yes        | 0.65               | 4.18               | 1 1/4 (+)                                | 2 (+)              |

## Legend

BEL = burned entire length

(+ ) = passed match test

(- ) = failed match test

## EXAMPLE V

This example illustrates certain preferred embodiments of the present invention employing cyanamide and methyl phosphonic acid (MPA) with one or more treatments (AATCC) procedure 34-1966 and the char length in inches is shown in TABLE I. (The greater the char length, the less the flame retardancy.)

Five pieces of cotton twill were dipped into an aqueous solution containing 18 weight percent methyl phosphonic acid, 16 weight percent cyanamide, 0.1 weight percent Triton X-100 non-ionic wetting agent and 5 weight percent Velvamine 380 polyethylene softener. The fabric samples were then dried in an oven for 10 minutes at 80°C and then cured in a second oven for 15 minutes at 160°C. The fabric samples were then washed, dried and conditioned as described in Example I except that the Sears detergent employed in Example II was used. One fabric sample was used as a control, while the remaining four fabric samples were subjected to from 1 to 4 retreatment operations with additional cyanamide.

20

TABLE V

| RETREATMENT OF MPA - CYANAMIDE TREATED FABRICS WITH ADDITIONAL CYANAMIDE |                        |                  |           |                    |           |          |           |           |           |
|--------------------------------------------------------------------------|------------------------|------------------|-----------|--------------------|-----------|----------|-----------|-----------|-----------|
| Run No.                                                                  | Number of Retreatments | Flame Retardance |           | Warp Shrinkage (%) |           | Ionicity |           | DP Rating |           |
|                                                                          |                        | 1 wash           | 50 washes | 1 wash             | 50 washes | 1 wash   | 50 washes | 1 wash    | 50 washes |
| 30 (control)                                                             | 0                      | 1 1/4 (+)        | BEL       | 8                  | 8         | 14       | 14        | 2         | 2         |
| 31                                                                       | 1                      | 2 (+)            | 1 1/4 (+) | 2.5                | 2.5       | 7        | 7         | 2         | 2         |
| 32                                                                       | 2                      | 1 1/2 (+)        | 1 1/2 (±) | 2                  | 2         | 6        | 6         | 2         | 2         |
| 33                                                                       | 3                      | 1 (+)            | 1 1/4 (±) | 1.5                | 1.5       | 4        | 4         | 2.5       | 2.5       |
| 34                                                                       | 4                      | 1 1/4 (+)        | 1 1/4 (+) | 1                  | 1         | 3.5      | 3.5       | 2         | 2         |

  

| Run No.      | Analyses |      |        |           | Ionicity |           |        |           | DP Rating |           |
|--------------|----------|------|--------|-----------|----------|-----------|--------|-----------|-----------|-----------|
|              | P(%)     | N(%) | 1 wash | 50 washes | 1 wash   | 50 washes | 1 wash | 50 washes | 1 wash    | 50 washes |
| 30 (control) | 2.89     | 2.73 | 0.64   | 0.53      | 0.75     | 0.74      | 2      | 2         | 2         | 2         |
| 31           | 2.95     | 2.78 | 1.38   | 1.13      | 0.56     | 0.60      | 3.5    | 2         | 2         | 2         |
| 32           | 2.92     | 2.74 | 1.83   | 1.51      | 0.44     | 0.52      | 4      | 2.5       | 2.5       | 2.5       |
| 33           | 2.93     | 2.75 | 2.16   | 1.75      | 0.37     | 0.47      | 4      | 3         | 3         | 3         |
| 34           | 2.98     | 2.81 | 2.48   | 1.97      | 0.33     | 0.46      | 4      | 3.5       | 3.5       | 3.5       |

cyanamide to improve durable fire retardancy (reduce 40 ionicity) and to improve also the durable press properties of the fabric. Each retreatment operation included souring the fabric sample with a dilute hydrochloric acid solution and then dipping the fabric sample into an aqueous solution containing 16 weight percent cyanamide, 0.1 weight percent Triton X-100 non-ionic wetting agent and 5 weight percent Velvamine 380 polyethylene softener. The fabric samples were then dried in an oven for 10 minutes at 80°C and then cured in a second oven for 15 minutes at 160°C. Each of the fabric samples were washed the indicated number of times in an automatic home laundering machine having one wash and two rinses with intermediate spin dry operations. Hard water was employed in the washes and rinses. In this example, the term "hard water" refers to 45 Irvine, Calif., water containing a degree of hardness 50 55

## EXAMPLE VI

This example illustrates certain preferred embodiments of the present invention employing cyanamide and methyl phosphonic acid with one or more diazomethane ( $\text{CH}_2\text{N}_2$ ) retreatments to improve durable flame retardance.

The procedure of Example V was repeated employing the same quantities of the same ingredients and the same times, procedures and conditions with the exception that diazomethane retreatments were used on two fabric samples instead of the cyanamide retreatment. The diazomethane retreatment consisted of soaking the soured fabric sample in an ether solution containing about 2.5 weight percent diazomethane for approximately 12 hours at about 25°C. The results are shown in TABLE VI.

TABLE VI

| THE EFFECT OF DIAZOMETHANE RETREATMENT (METHYLATION) ON MPA - CYANAMIDE TREATED FABRICS |                                              |                  |           |          |           |          |        |           |      |
|-----------------------------------------------------------------------------------------|----------------------------------------------|------------------|-----------|----------|-----------|----------|--------|-----------|------|
| Run No.                                                                                 | Number of $\text{CH}_2\text{N}_2$ Treatments | Flame Retardance |           | Ionicity |           | Analyses |        |           |      |
|                                                                                         |                                              | 1 wash           | 50 washes | 1 wash   | 50 washes | P(%)     | 1 wash | 50 washes | N(%) |
| 35 (control)                                                                            | 0                                            | 2 (+)            | —         | 0.73     | —         | 2.69     | —      | 0.57      | —    |
| 36                                                                                      | 1                                            | 2 (+)            | 2 (±)     | 0.39     | 0.40      | —        | —      | —         | —    |
| 37                                                                                      | 2                                            | 2 (+)            | 2 (±)     | 0.07     | 0.12      | 2.64     | 2.63   | 0.47      | 0.45 |

## EXAMPLES VII - VIII

These examples illustrate certain preferred embodiments of the present invention employing cyanamide with methyl phosphonic acid on wool (runs 38 and 39) and on rayon (run 40) fabrics.

The procedure of Example I (run 2) is repeated employing the same quantities of the same ingredients and

dures and conditions with the exception that the pH of the phosphonic acid-containing pad bath was adjusted to a pH of 3 using ammonium hydroxide; mercerized flannel was used instead of cotton twill; and the hardness equivalent of the wash and rinse water was 40 ppm calcium carbonate (Menlo Park, California). The resulting flame retardancy values are shown in TABLE X.

TABLE X

## RETREATMENT OF MPA - CYANAMIDE TREATED FABRICS WITH ADDITIONAL CYANAMIDE

| Run No. | Number of Retreatments | Flame Retardance after Indicated Number of Washes AATCC 34-1966 (length of char) |                    |
|---------|------------------------|----------------------------------------------------------------------------------|--------------------|
|         |                        | One Wash (in.)                                                                   | Fifty Washes (in.) |
| 45      | 0                      | 1 1/4 (±)                                                                        | BEL                |
| 46      | 1                      | 1 3/4 (+)                                                                        | 2 1/2 (±)          |

the same times, procedures and conditions with the exception that the cotton twill was replaced by bleached, undyed wool in run 38, by dyed wool (grey) in run 39, and by rayon twill in run 40. The results are recorded in TABLE VII.

TABLE VII

## TREATMENT OF WOOL AND RAYON WITH MPA - CYANAMIDE (1:2)

| Run No. | Fabric                | Add-On | Flame Retardance |           |           |           |
|---------|-----------------------|--------|------------------|-----------|-----------|-----------|
|         |                       |        | 1 wash           | 5 washes  | 10 washes | 50 washes |
| 38      | Bleached, undyed wool | 11.2%  | 1 1/4 (+)        | 1 (+)     | —         | —         |
| 39      | Dyed Wool (grey)      | 13.5%  | 2 1/2 (+)        | 3 (+)     | 5 (+)     | —         |
| 40      | Rayon twill           | 18.9%  | 1 1/2 (±)        | 1 3/4 (±) | 2 (—)     | 2 1/4 (—) |

## EXAMPLE IX

This example illustrates the present invention when cyanamide and methyl phosphonic acid are applied to a fabric from a pad bath which also contains ammonium hydroxide to increase the otherwise autogenous pH of the bath to a pH of 5, and the results that are achieved using various curing times.

The procedure of Example II was repeated employing the same quantities of the same ingredients and the same times, procedures and conditions with the exception that the pH of the pad bath in each run was adjusted to a pH of 5 with ammonium hydroxide, and the fabric samples were dried at about 65°C for 8 minutes and cured at about 160°C for various times as shown in TABLE IX. The resulting flame retardancy values are also shown in TABLE IX.

As may be seen from TABLE IX, good flame retardancy was achieved in all runs.

35 methylol compound to improve the durability of the flame retardancy.

The procedure of Example V is repeated employing the same quantities of the same ingredients and the same times, procedures and conditions with the exception that the cyanamide is replaced with a N-methylol compound in the retreatment bath (16% Aerotex 92 methylolated melamine).

Further improvement in durability of flame retardancy is observed.

45 The principles, preferred embodiments and modes of operation of the present invention have been described in the foregoing specification. The invention which is intended to be protected herein, however, is not to be construed as limited to the particular forms disclosed, since these are to be regarded as illustrative rather than restrictive. Variations and changes may be made by those skilled in the art without departing from the spirit of the present invention.

TABLE IX

## FLAME RETARDANCE OF METHYL PHOSPHONIC ACID:CYANAMIDE SYSTEMS AT VARYING CURE TIMES

| Run No. | pH of Bath | Curing Times (min.) | Flame Retardance after Indicated Number of Washes AATCC 34-1966 (length of char) |                    |
|---------|------------|---------------------|----------------------------------------------------------------------------------|--------------------|
|         |            |                     | One Wash (in.)                                                                   | Fifty Washes (in.) |
| 41      | 5          | 2.5                 | 3 (+)                                                                            | 3 (—)              |
| 42      | 5          | 5                   | 2 1/2 (+)                                                                        | 2 1/2 (—)          |
| 43      | 5          | 10                  | 2 3/4 (+)                                                                        | 2 3/4 (—)          |
| 44      | 5          | 15                  | 2 1/2 (+)                                                                        | 2 3/4 (—)          |

## EXAMPLE X

Example V was repeated employing the same quantities of the same ingredients and the same times, proce-

We claim:

1. A process for rendering cellulosic and wool fiber-containing material flame retardant, which process comprises

contacting the material with cyanamide and at least one phosphonic acid represented by the structural formula:



5

wherein  $\text{R}^1$  represents a monovalent radical selected from the group consisting of hydrogen and lower alkoxyl; and wherein  $\text{R}^2$  represents a monovalent radical selected from the group consisting of hydrogen and lower alkyl, to deposit on the material a flame retarding amount of the phosphonic acid with cyanamide.

2. A process according to claim 1 wherein the material is cellulosic and the phosphonic acid is methyl phosphonic acid.

3. A process according to claim 1 for rendering cellulosic fiber-containing material flame retardant, which process comprises

contacting and fixing on the material with cyanamide a flame retarding amount of at least one phosphonic acid represented by the structural formula:



25

wherein  $\text{R}^1$  represents a monovalent radical selected from the group consisting of hydrogen and methoxyl; and wherein  $\text{R}^2$  represents a monovalent radical selected from the group consisting of hydrogen and methyl; and wherein during contacting the molar ratio of phosphonic acid to cyanamide is from 1:10 to 10:1.

4. A process according to claim 3 wherein the material is fixed by heating the material for a period of time and at a temperature at least sufficient to give an add-on of from 1 to 30 percent; wherein the phosphonic acid and cyanamide are in solution when contacted with the material; wherein the pH at fixation is less than 2.5; and wherein the cellulosic fiber-containing material is cotton cloth.

5. A process according to claim 3 wherein the cellulosic fiber-containing material is fixed by contacting the material with the phosphonic acid and cyanamide and then heating the material at a temperature between about 100° and 300°C.

6. A process for rendering cellulosic textile material flame retardant comprising in sequence the steps of:

I. contacting the material with an aqueous solution of cyanamide and at least one phosphonic acid selected from the group consisting of methyl phosphonic acid and methyl phosphonic acid mono-methyl ester, wherein the molar ratio of phosphonic acid:cyanamide is 1:10 to 10:1, and

II. heating the material to fix the phosphonic acid with cyanamide on the material to give an add-on of between about 1 and 30 percent.

7. A process according to claim 6 for rendering cellulosic fiber-containing textile material durably flame retardant, which process comprises in sequence the steps of:

I. contacting the material with an aqueous mixture of cyanamide and methyl phosphonic acid wherein

the molar ratio of phosphonic acid:cyanamide is 1:10 to 10:1, and;

II. fixing the retardancy in the material at a pH less than 2.5 by heating the material until an add-on of between about 1 and 30 percent is achieved and the flame retardancy becomes durable to at least 30 hard water washes.

8. A process according to claim 7 wherein the cellulosic material is mercerized cotton cloth and the flame retardancy is durable to at least 50 hard water washes.

9. A process according to claim 7 wherein the aqueous mixture of cyanamide and methyl phosphonic acid further contains ammonium hydroxide, and an ammonium salt of the phosphonic acid is deposited on the textile material.

10. A process for rendering cellulosic and wool fiber-containing material durably flame retardant, which process comprises the steps of:

I. contacting the material with cyanamide and at least one phosphonic acid represented by the structural formula:



25

wherein  $\text{R}^1$  represents a monovalent radical selected from the group consisting of hydrogen and lower alkoxyl; and wherein  $\text{R}^2$  represents a monovalent radical selected from the group consisting of hydrogen and lower alkyl, to deposit on the material a flame retarding amount of the phosphonic acid with cyanamide; and subsequently,

II. contacting the material with at least one member selected from the group consisting of cyanamide, diazomethane and water-soluble compounds possessing reactive N-methylol groups, in an amount sufficient to improve the durability of the flame retardancy of the material to repeated hard water washing.

30

11. A process according to claim 10 wherein in step (I) the phosphonic acid and the cyanamide are in solution when contacted with the material and the molar ratio of phosphonic acid to cyanamide is from 1:10 to 10:1; and in step (II) the cyanamide is in solution when contacted with the material, and the material is thereafter heated to give a total add-on of from 1 to 30 percent.

35

12. A process for rendering cellulosic textile material durably flame retardant and wrinkle resistant, which process comprises the steps of:

I. contacting the material with an aqueous mixture of cyanamide and at least one phosphonic acid selected from the group consisting of methyl phosphonic acid and methyl phosphonic acid mono-methyl ester, wherein the molar ratio of phosphonic acid:cyanamide is 1:10 to 10:1, and

II. heating the material to fix at a pH less than 2.5 the phosphonic acid with cyanamide on the material to give and add-on of between about 1 and 30 percent, and

III. contacting the material with an aqueous solution of cyanamide and heating the material to improve the durability of the flame retardancy, dimensional stability, and durable press properties of the material.

13. A process according to claim 12 for rendering cotton fiber-containing textile material durably flame

40

45

50

55

60

65

retardant and for simultaneously improving the dimensional stability and durable press properties of the textile material, which process comprises in sequence the steps of:

- I. contacting the material with an aqueous solution of cyanamide with methyl phosphonic acid wherein the molar ratio of phosphonic acid:cyanamide is 1:10 to 10:1, 5
- II. fixing the retardancy in the material at a pH less than 1.5 by heating the material until an add-on of between about 1 and 30 percent is achieved and the flame retardancy becomes durable to at least 30 hard water washes; and
- III. regenerating an acid form of fixed phosphonic acid residue on the material and then contacting 15 the material with an aqueous solution of cyanamide and heating the material to improve the durability of the flame retardancy to at least 50 hard water washes, and to improve dimensional stability, and durable press properties of the material.

14. A process for rendering cellulosic textile material durably flame retardant, which process comprises the steps of:

- I. contacting the material with an aqueous mixture of cyanamide and at least one phosphonic acid selected from the group consisting of methyl phosphonic acid and methyl phosphonic acid mono-methyl ester, wherein the molar ratio of phosphonic acid:cyanamide is 1:10 to 10:1, and 25
- II. heating the material to fix the phosphonic acid at a pH less than 2.5 with cyanamide on the material to give an add-on of between about 1 and 30 percent, and
- III. contacting the material with an aqueous solution of at least one water-soluble compound possessing 30 reactive N-methylol groups and curing the material to improve the durability of the flame retardancy of the material.

20

35

15. A process according to claim 14 for rendering cotton fiber-containing textile material durably flame retardant, which process comprises in sequence the steps of:

- I. contacting the material with an aqueous solution of cyanamide with methyl phosphonic acid wherein the molar ratio of phosphonic acid:cyanamide is 1:10 to 10:1,
- II. fixing the retardancy in the material at a pH less than 1.5 by heating the material until an add-on of between about 1 and 30 percent is achieved and the flame retardancy becomes durable to at least 30 hard water washes; and
- III. regenerating an acid form of fixed phosphonic acid residue on the material and then contacting the material with an aqueous solution of the N-methylol compound, and heating the material to cure and the durability of the flame retardancy is improved to at least 50 hard water washes.

16. A process according to claim 15 wherein the textile material is mercerized cotton cloth, and wherein the aqueous mixture of cyanamide and methyl phosphonic acid further contains ammonium hydroxide, and an ammonium salt of the phosphonic acid is deposited on the textile material.

17. A flame retardant material produced according to the process of claim 1.

18. A durably flame retardant material produced according to the process of claim 7.

19. A durably flame retardant material produced according to the process of claim 10.

20. A durably flame retardant and wrinkle resistant material produced according to the process of claim 13.

21. A durably flame retardant material produced according to the process of claim 15.

\* \* \* \* \*

40

45

50

55

60

65